

# UNITED STATES PATENT OFFICE.

HANS BORGmann, OF NEW YORK, N. Y.

## PAINT-VEHICLE.

SPECIFICATION forming part of Letters Patent No. 387,488, dated August 7, 1883.

Application filed July 28, 1887. Serial No. 245,547. (No specimens.)

*To all whom it may concern:*

Be it known that I, HANS BORGmann, a citizen of the German Empire, residing at New York, in the county and State of New York, 5 have invented new and useful Improvements in Fixing Colors, of which the following is a specification.

The object of this invention is to provide a composition of matter to be used for fixing water-color.

My composition consists of the following ingredients, combined in substantially the proportions stated, namely: one hundred parts, by weight, of alkali solution; one hundred parts, 15 by weight, of water; ten to twenty parts, by weight, of caseine solution; twenty to forty parts, by weight, of an oily or oleaginous body. These ingredients are to be thoroughly mingled by heating and agitation.

20 The alkali solution which I use is a soda or potash solution, which I form by dissolving one part, by weight, of soda or potash in one hundred parts, by weight, of water.

The caseine solution is prepared by mixing 25 caseine with one per cent., by weight, of alcohol.

The oily or oleaginous body which I employ is balsamic resin, wax, or fat, or a mixture of two or more of these substances. The proportion of the balsamic resin, wax, and fat, among 30 themselves, depends upon the desired hardness or softness of the binding material and upon the depth or warmth of color which the binding material is to impart to the painting. By increasing the amount of resin the hardness is increased, and by increasing the amount of wax the softness is increased. By increasing the amount of fat the depth or warmth of color of the painting is increased.

I have found it an advantage in forming the 35 caseine solution to add shellac to said solution,

as thereby the hardness and durability of the binding material are increased, and I have at times used as much as equal parts of shellac and caseine; but, if desired, said shellac may be omitted and the caseine be employed without the addition of shellac. 45

The binding material above described is spread over the painting or drawing after said painting or drawing has been completed. An ordinary brush will serve for spreading the 50 binding material over the painting. After the binding material has been spread over the painting or drawing said binding material is allowed to dry, after which any excess of soluble matter which may be on the surface of the 55 binding material can be removed by washing with water.

I have found my binding material to be very effective when used on colors of metallic oxide and of alkaline earths, or when the colors are 60 applied to a foundation composed of mortar, lime, wall-glued chalk or clay, or of gypsum saturated with baryta-water.

Instead of spreading the binding material over the finished painting or drawing, the 65 binding material may be mixed with a solution of the color, and the color and binding material thus be simultaneously applied.

What I claim is—

A binding material for water-color, consisting of alkali, water, caseine, and an oleaginous body, substantially in the proportions specified. 70

In testimony whereof I have hereunto set my hand and seal in the presence of two subscribing witnesses. 75

HANS BORGmann. [L. S.]

Witnesses:

W. C. HAUFF,

E. F. KASTENHUBER.